

M. M. MERRITT,  
ELECTROLYTICALLY COATED WIRE,  
APPLICATION FILED OCT. 7, 1919.

1,405,534.

Patented Feb. 7, 1922.



*Inventor:  
Matthew M. Merritt,  
by Emery Booth James, Varney.  
Atty's.*

# UNITED STATES PATENT OFFICE.

MATTHEW M. MERRITT, OF SOUTH MIDDLETON, MASSACHUSETTS, ASSIGNOR TO  
MERRITT METALS COMPANY, OF SALEM, MASSACHUSETTS, A CORPORATION OF  
MASSACHUSETTS.

## ELECTROLYTICALLY-COATED WIRE.

1,405,534.

Specification of Letters Patent.

Patented Feb. 7, 1922.

Original application filed April 15, 1919, Serial No. 290,152. Divided and this application filed October 7, 1919. Serial No. 329,000.

To all whom it may concern:

Be it known that I, MATTHEW M. MERRITT, a citizen of the United States, and a resident of South Middleton, county of Essex, State 5 of Massachusetts, have invented an Improvement in Electrolytically-Coated Wire, of which the following description, in connection with the accompanying drawings, is a specification, like characters on the drawings 10 representing like parts.

This invention pertains to improvements in electrolytically coated wire. It is among the objects of the invention to provide a wire having a copper exterior shell of a superior 15 quality.

This application is a divisional of my co-pending application Serial No. 290,152, filed April 15, 1919, which matured into United, States Patent No. 1,322,494, dated November 18th, 1919, to which reference should be 20 made for the preferred apparatus and method used in connection with the production of the preferred form of wire to which this application is specifically directed.

In the drawing which forms part of this specification, the figure is a cross-section of a preferred form of electrolytically coated wire.

Referring to the drawing and to the preferred form of my invention selected for 30 illustrative purposes, I have shown a wire 2, which may be of aluminum and which, as described in my co-pending application above referred to, has its surface treated, 35 preferably, in such a way as to remove the oxide on the surface thereof and preferably to deposit a film of foreign substance thereon to serve as an oxide-excluding medium over the surface of the aluminum and to provide 40 a surface thereto other than aluminum which will readily take in a satisfactory manner the deposit of copper or other metal during subsequent electro-deposition. The oxide-

excluding medium is preferably tin and is illustrated in the drawing by the ring 3, of 45 which the thickness is greatly exaggerated so that it will show clearly in the drawing. This oxide-excluding medium, preferably of tin, may be applied by a combined deoxidizing and tinning operation by treating the 50 surface of the aluminum wire with a mixture of muriatic acid, water and tin chloride. The interposition of the coating of oxide-excluding medium between the aluminum and the copper shell 4 minimizes that galvanic 55 deterioration of these metals which normally arises where, in the presence of even a trace of moisture, copper and aluminum are permitted to come into contact or even into close proximity.

Where the wire forming the core is of ferrous material, the exterior coating corresponding to the coating 3 may be an electrolytic, alkaline copper deposit, the exterior deposit forming the wire 4 being electrolytic 65 acid copper. This construction is claimed in a divisional application Serial No. 505,371, filed October 4th, 1921.

While I have shown in the drawing and described rather specifically preferred forms 70 of my invention, it will be understood that considerable changes may be made without departing from the scope of my invention, which is best defined in the following claims.

1. Wire comprising a core of aluminum, a 75 film of oxide-excluding material surrounding said core of aluminum and a shell of copper surrounding said oxide-excluding film.

2. Wire comprising a core of aluminum, a 80 film of tin surrounding said core of aluminum and a shell of copper surrounding said tin film.

In testimony whereof, I have signed my name of this specification.

MATTHEW M. MERRITT.